# EUROPEAN PATENT SPECIFICATION

(11) **EP 3 095 887 B1**
(45) Date of publication and mention of the grant of the patent: **13.03.2019**
(21) Application number: 15737102.2
(22) Date of filing: 08.01.2015
(51) Int. Cl.: C22C 38/00, C21D 8/12, C21D 9/46, C22C 38/60, H01F 1/16, C22C 38/02, C22C 38/04, C22C 38/06, H01F 1/04

(54) **NON-ORIENTED ELECTRICAL STEEL SHEET HAVING EXCELLENT MAGNETIC PROPERTIES**
UNGERICHTETES ELEKTROSTAHLBLECH MIT HERVORRAGENDEN MAGNETISCHEN EIGENSCHAFTEN
FEUILLE D'ACIER ÉLECTRIQUE NON DIRECTIONNEL PRÉSENTANT D'EXCELLENTES PROPRIÉTÉS MAGNÉTIQUES

(30) Priority: 14.01.2014 JP 2014003983
(43) Date of publication of application: 23.11.2016
(73) Proprietor: JFE Steel Corporation, Tokyo 100-0011 (JP)
(72) Inventor: ODA Yoshihiko, Tokyo 100-0011 (JP); NAKANISHI Tadashi, Tokyo 100-0011 (JP); KOSEKI Shinji, Tokyo 100-0011 (JP); OKUBO Tomoyuki, Tokyo 100-0011 (JP)
(74) Representative: Haseltine Lake LLP
(86) International application number: PCT/JP2015/050317
(87) International publication number: WO 2015/107967

(56) References cited:
- WO-A1-2013/137092
- JP-A- H0 673 511
- JP-A- H0 860 311
- JP-A- 2001 158 950
- JP-A- 2001 192 788
- JP-A- 2001 323 344
- JP-A- 2004 292 829
- JP-A- 2006 104 530
- JP-A- 2006 104 530
- JP-A- 2008 231 504
- JP-A- 2008 231 504
- JP-A- 2013 189 693
- JP-A- 2013 192 417

## Description

### TECHNICAL FIELD

This invention relates to a non-oriented electrical steel sheet having excellent magnetic properties, and more particularly to a non-oriented electrical steel sheet having a high magnetic flux density.

### RELATED ART

Recently, high-efficiency induction motors are used in view of the increasing demand for energy-saving. In order to improve the efficiency of the high-efficiency induction motor, a laminate thickness of a core is made thick, or a filling rate of winding wires is increased, or an electrical steel sheet used as a core is exchanged from the conventional low-grade material to a high-grade material having a lower iron loss.

A core material used in the induction motor is required to be low in not only the iron loss but also the effective excitation current at a predetermined magnetic flux density for lowering the effective excitation current to decrease copper loss. In order to reduce the excitation current, it is effective to increase a magnetic flux density of the core material. Further, a driving motor used in hybrid cars and electric cars, which is becoming popular rapidly, is necessary to have a high torque at startup and during acceleration, so that it is desired to further increase a magnetic flux density.

As an electrical steel sheet having an increased magnetic flux density, for example, Patent Document 1 discloses a non-oriented electrical steel sheet in which 0.1-5 mass% of Co is added to a steel having not more than 4 mass% of Si. Further disclosures of non-oriented electrical steel sheet includes: Patent Document 2, wherein a motor core having a small hysteresis loss and good magnetic characteristics is disclosed; Patent Document 3, wherein a method of producing a non-oriented electrical steel sheet with a high magnetic flux density and low iron loss is disclosed; and Patent Documents 4, wherein a method for producing non-oriented electrical steel sheets suitable for use as a core material of a motor is disclosed.

### PRIOR ART DOCUMENTS

### PATENT DOCUMENT

Patent Document 1: JP-A-2000-129410
Patent Document 2: JP-A-2013-192417
Patent Document 3: WO 2012/137092
Patent Document 4: JP-A-2006-104530

### SUMMARY OF THE INVENTION

### TASK TO BE SOLVED BY THE INVENTION

However, since Co is a very expensive element, if the technique
disclosed in Patent Document 1 is applied to an ordinary motor, there is a problem that the raw material cost is extraordinarily increased. Therefore, it is desired to develop a method for increasing the magnetic flux density of the electrical steel sheet without increasing the raw material cost.

The invention is made in view of the above problem inherent to the conventional art, and an object thereof is to provide a non-oriented electrical steel sheet having a high magnetic flux density and a low iron loss cheaply and stably.

### SOLUTION FOR TASK

The inventors have made various studies for solving the above task. As a result, it has been found that a magnetic flux density can be largely increased by decreasing Se inevitably incorporated into a steel having a reduced A1 content and an added P content to an ultralow level, and the invention has been accomplished.

That is, the invention is a non-oriented electrical steel sheet having a chemical composition as defined in claims 1 and 2.

Further, the non-oriented electrical steel sheet according to the invention is characterized in that a sheet thickness is 0.05-0.30 mm.

### EFFECT OF THE INVENTION

According to the invention, a non-oriented electrical steel sheet having a high magnetic flux density can be provided cheaply and stably, so that it can be preferably used as a core material for a high-efficiency induction motor, a driving motor of a hybrid car and an electric car requiring a high torque, and a high-efficiency electric generator requiring a high generation efficiency.

### BRIEF DESCRIPTION OF THE DRAWINGS

FIG. 1 is a graph showing an influence of P content upon a magnetic flux density B₅₀ after a finish annealing.
FIG. 2 is a graph showing an influence of Se content upon a magnetic flux density B₅₀ after a finish annealing.

### EMBODIMENTS FOR CARRYING OUT THE INVENTION

Hereinafter, experiments building a momentum on the development of the invention will be described.

### <Experiment 1>

At first, in order to investigate an influence of P upon a magnetic flux density, steels prepared by adding P variously changed within a range of tr.-0.16 mass% to an Al-less steel containing C: 0.0020 mass%, Si: 3.07 mass%, Mn: 0.24 mass%, Al: 0.001 mass% and N: 0.0021 mass%, P:0.01 mass% and S: 0.0021 mass% and an Al-added steel containing C: 0.0022 mass%, Si: 2.70 mass%, Mn: 0.24 mass%, Al: 0.30 mass% and N: 0.0018 mass%, P: 0.01 mass% and S: 0.0013 mass% are melted in a laboratory to form steel ingots, which are hot rolled to form hot rolled sheets of 1.6 mm in thickness. Thereafter, the hot rolled sheets are subjected to a hot band annealing at 980°C for 30 seconds, pickled and cold rolled to form cold rolled sheets having a thickness of 0.20 mm, which are further subjected to a finish annealing at 1000°C in an atmosphere of 20 vol% H₂ - 80 vol% N2 for 10 seconds.

From the cold rolled and annealed sheets thus obtained are cut out test specimens with a width of 30 mm and a length of 280 mm in a rolling direction (L-direction) and in a direction perpendicular to the rolling direction (C-direction) as a length direction, respectively, to measure a magnetic flux density B₅₀ by a 25 cm Epstein method described in JIS C2550, the results of which are shown in FIG. 1 as a relation to P content. As seen from FIG.1, an improvement of the magnetic flux density is not recognized in the Al-added steel even when P content is increased, whereas the magnetic flux density is improved in the Al-less steel with an increase of P content.

The reason why the magnetic flux density is improved with an increase of P content in the Al-less steel as described above is not sufficiently clear at present, but it is considered that Al somewhat affects the segregation behavior of P before the cold rolling and the diffusion rate of P is increased by containing no Al to promote the segregation of P into the crystal grain boundary to thereby improve the texture.

### <Experiment 2>

Then, in order to investigate the production stability of P-added steel, an Al-less steel containing C: 0.0018 mass%, Si: 3.10 mass%, Mn: 0.20 mass%, Al: 0.001 mass%, N: 0.0015 mass%, P: 0.06 mass% and S: 0.0014 mass% is tapped at 10 charges and hot rolled to form hot rolled sheets of 1.6 mm in thickness. The hot rolled sheets are subjected to a hot band annealing at 980 °C for 30 seconds, pickled and cold rolled to obtain cold rolled sheets each having a thickness of 0.20 mm, which are subjected to a finish annealing at 1000 °C in an atmosphere of 20 vol% H₂ - 80 vol% N₂ for 10 seconds to obtain cold rolled and annealed sheets.

When the magnetic flux density B₅₀ is measured as to the cold rolled and annealed sheets thus obtained in the same way as in the above experiment, it becomes clear that the measured results are largely varied. As a composition analysis is performed in steel sheets having a low magnetic flux density, it is found that Se is included in an amount of 0.0022-0.0035 mass%. From this result, it is inferred that Se is segregated into the grain boundary to suppress the segregation of P into the grain boundary and hence the magnetic flux density is decreased. It is thought that Se is an element contained in a scrap or the like and is incorporated inevitably with the increase of the use rate of the scrap in recent years.

### <Experiment 3>

Therefore, in order to investigate an influence of Se upon the magnetic flux density, steels prepared by adding Se variously changed within a range of tr.-0.007 mass% to a steel containing C: 0.0013 mass%, Si: 3.21 mass%, Mn: 0.15 mass%, Al: 0.002 mass% and N: 0.0018 mass%, P: 0.05 mass% and S: 0.0009 mass% are melted in a laboratory to form steel ingots, which are hot rolled to form hot rolled sheets of 1.6 mm in thickness. Then, the hot rolled sheets are subjected to a hot band annealing at 1000 °C for 30 seconds, pickled and cold rolled to obtain cold rolled sheets each having a thickness of 0.20 mm, which are subjected to a finish annealing at 1000 °C in an atmosphere of 20 vol% H₂ - 80 vol% N₂ for 10 seconds.

From the cold rolled and annealed sheets are cut out test specimens with a width of 30 mm and a length of 280 mm to measure a magnetic flux density B₅₀ in the same way as in the above experiment. The results are shown in FIG. 2 as a relation to Se content. As seen from FIG.2, the magnetic flux density is decreased when Se content exceeds 0.0020 mass%, and hence it is necessary to restrict the Se content to not more than 0.0020 mass%.

The invention is based on the above new knowledge.

The chemical composition in the non-oriented electrical steel sheet according to the invention will be described below.

### C: not more than 0.010 mass%

Since C is a harmful element deteriorating the iron loss, less amount is more preferable. When C exceeds 0.010 mass%, the iron loss is remarkably increased by magnetic aging, so that the upper limit of C is 0.010 mass%. Preferably, it is not more than 0.005 mass%. Also, less amount of C is more preferable and therefore a lower limit is not particularly limited.

### Si: 1-4 mass%

Si is an element generally added as a deoxidizing agent of steel. In electrical steel sheets, however, it is an important element having an effect of increasing an electrical resistance to decrease an iron loss at a high frequency, so that it is necessary to add in an amount of not less than 1 mass% in order to obtain such an effect. However, when it exceeds 4 mass%, an excitation effective current is considerably increased, so that the upper limit is set to 4 mass%. Preferably, it is a range of 1.0-3.5 mass%.

### Mn: 0.05-3 mass%

Mn has an effect of preventing a hot brittleness during the hot rolling of steel to prevent the generation of surface defects, so that it is added in an amount of not less than 0.05 mass%. On the other hand, as Mn content becomes higher, the magnetic flux density and the saturated magnetic flux density are decreased, so that the upper limit of Mn content is set to 3 mass%. Preferably, it is a range of 0.1-1.7 mass%.

### Al: not more than 0.004 mass%

When Al is decreased, the texture of the finish-annealed steel sheet can be improved to increase the magnetic flux density. Also, the decrease of Al is necessary for promoting the grain boundary segregation of P to increase the magnetic flux density. When it exceeds 0.004 mass%, such an effect cannot be obtained. Accordingly, the upper limit of Al is set to 0.004 mass%. Preferably, it is not more than 0.002 mass%. Moreover, the lower limit of Al is not particularly limited because less amount is more preferable.

### N: not more than 0.005 mass%

N forms a nitride to deteriorate magnetic properties, so that it is limited to not more than 0.005 mass%. Preferably, it is not more than 0.002 mass%. The lower limit is not particularly limited because less amount is more preferable.

### P: 0.03-0.20 mass%

P is one of important elements in the invention and has an effect of increasing the magnetic flux density by segregation into the grain boundary in the Al-less steel as shown in FIG. 1. Such an effect is obtained with an addition of not less than 0.03 mass%. While, when it exceeds 0.20 mass%, it is difficult to perform cold rolling. In the invention, therefore, the addition amount of P is in a range of 0.03-0.20 mass%. Preferably, it is in a range of 0.05-0.10 mass%.

### S: not more than 0.01 mass%

S is an element forming a sulfide such as MnS or the like to deteriorate magnetic properties of a product, so that less amount is more preferable. In the invention, therefore, the upper limit of S is set to 0.01 mass% in order not to deteriorate the magnetic properties. It is preferably not more than 0.005 mass%, more preferably not more than 0.001 mass% from a viewpoint of promoting the grain boundary segregation of P. Moreover, the lower limit is not particularly limited because less amount is more preferable.

### Se: not more than 0.002 mass%

Since Se is a harmful element segregating into the grain boundary earlier than P to suppress the grain boundary segregation of P and decrease the magnetic flux density, so that it is necessary to decrease Se as much as possible. In the invention, therefore, the upper limit is set to 0.002 mass%. Preferably, it is not more than 0.001 mass%.

However, Sn and Sb described later have an effect of inhibiting the harmful effect of Se, so that when Sn and Sb are added, the upper limit of Se can be expanded to 0.003 mass%. In this case, Se is preferably not more than 0.0025 mass%.

The non-oriented electrical steel sheet according to the invention may contain one or more selected from Sn, Sb and Ca within the following range in addition to the above essential ingredients and Mg.

### Sn: 0.001-0.1 mass%

Sn is an element segregating into the grain boundary, but is little in the influence on P segregation and rather has an effect of accelerating formation of a deformable band inside grains to increase the magnetic flux density. Such an effect is obtained with an addition of not less than 0.001 mass%. While, when it is added in an amount exceeding 0.1 mass%, embrittlement of steel is caused to increase surface defects such as fracture of the sheet, scab and the like in the production process. Therefore, when Sn is added, it is preferable to be a range of 0.001-0.1 mass%. More preferably, it is a range of 0.001-0.06 mass%.

### Sb: 0.001-0.1 mass%

Sb is an element segregating into the grain boundary like Sn, but is little in the influence on P segregation and rather has an effect of suppressing nitriding in the annealing to improve the magnetic properties. Such an effect is obtained with an addition of not less than 0.001 mass%. On the other hand, when it is added in an amount exceeding 0.1 mass%, embrittlement of steel is caused to increase surface defects such as fracture of the sheet, scab and the like in the production process. Therefore, when Sb is added, it is preferable to be a range of 0.001-0.1 mass%. More preferably, it is a range of 0.001-0.06 mass%.

### Ca: 0.001-0.005 mass%

Ca has an effect of coarsening a sulfide to decrease an iron loss, so that it can be added in an amount of not less than 0.001mass%. On the other hand, if it is exceedingly added, the above effect is saturated and brings disadvantageous economically. Therefore, the upper limit is set to 0.005 mass%. More preferably, it is a range of 0.001-0.003 mass%.

### Mg: 0.001-0.005 mass%

Mg has an effect of coarsening a sulfide to decrease an iron loss like Ca, so that it is added in an amount of not less than 0.001mass%. On the other hand, if it is exceedingly added, the above effect is saturated and brings disadvantageous economically. Therefore, the upper limit is set to 0.005 mass%. More preferably, it is in a range of 0.001-0.003 mass%.

The remainder other than the above ingredients in the non-oriented electrical steel sheet according to the invention is Fe and inevitable impurities. However, an addition of other elements may not be refused within a range not damaging the effect of the invention.

Next, the thickness (product thickness) of the non-oriented electrical steel sheet according to the invention will be described below.

The thickness of the non-oriented electrical steel sheet according to the invention is preferable to be not more than 0.30 mm from a viewpoint of reducing an iron loss at a high frequency zone. While, when the thickness is less than 0.05 mm, there are caused such problems that the lamination number required for the production of an iron core is increased and the rigidity of the steel sheet is extremely decreased to increase vibration of a motor and so on. Therefore, the thickness is preferable to be a range of 0.05-0.30 mm. More preferably, it is a range of 0.10-0.20 mm.

Next, the method of producing the non-oriented electrical steel sheet according to the invention will be described.

In the non-oriented electrical steel sheet according to the invention, a well-known production method for a non-oriented electrical steel sheet can be used as long as a slab containing Al, P and Se in the above-described proper ranges is used as a raw material thereof and is not particularly limited. For example, there can be adopted the following method or a method in which a steel adjusted to have a predetermined chemical composition is melted by a refining process such as a converter, electric furnace or the like, subjected to a secondary refining with a degassing device or the like and continuously casted to obtain a steel slab, which is subjected to hot rolling, hot band annealing as required, pickling, cold rolling, finish annealing and further coating and baking of an insulating film.

Moreover, when the hot band annealing is performed, a soaking temperature is preferable to be in a range of 900-1200°C. When it is lower than 900°C, the effect by the hot band annealing cannot be sufficiently obtained and the magnetic properties are not improved, while when it exceeds 1200°C, the cost becomes disadvantageous and the grain size in the hot rolled sheet becomes coarsened to bring about a fear of causing a breakage in the cold rolling.

Also, the cold rolling of the hot rolled sheet to a final thickness is preferable to be once or twice or more including intermediate annealing therebetween. Particularly, the final cold rolling is preferable to be a warm rolling at a sheet temperature of approximately 200°C unless there is a problem in equipment, production constraint or cost, because the warm rolling has a large effect of increasing the magnetic flux density.

The finish annealing applied to the cold rolled sheet with a final thickness is preferably a continuous annealing of soaking at a temperature of 900-1150°C for 5-60 seconds. When the soaking temperature is lower than 900°C, recrystallization is not sufficiently advanced and good magnetic properties cannot be obtained. While, when it exceeds 1150°C, crystal grains are coarsened and the iron loss particularly at a high frequency zone is increased.

It is preferable that an insulation coating is formed on the surface of the steel sheet after the finish annealing in order to decrease the iron loss. As the insulation coating is desirably used a semi-organic insulation coating containing a resin in order to ensure a good punchability.

The non-oriented electrical steel sheet thus produced may be used without stress-relief annealing or may be used after the stress-relief annealing. Alternatively, the stress relief annealing may be conducted after the shaping through a punching process. Here, the stress relief annealing is generally conducted at 750°C for 2 hours.

### EXAMPLE

A steel having a chemical composition as shown in Table 1 and the remainder being Fe and inevitable impurities is melted and continuously casted to obtain a steel slab, which is heated at a temperature of 1140°C for 1 hour and subjected to hot rolling at a finish rolling end temperature of 800°C and a coiling temperature of 610°C to obtain a hot rolled sheet having a thickness of 1.6 mm. The hot rolled sheet is subjected to a hot band annealing at 1000°C for 30 seconds and then cold rolled to obtain a cold rolled sheet having a thickness shown in Table 1. Subsequently, the cold rolled sheet is subjected to a finish annealing of holding a temperature shown in Table 1 for 10 seconds to obtain a cold rolled and annealed sheet (non-oriented electrical steel sheet).

From the cold rolled and annealed sheet thus obtained are cut out Epstein test specimens with a width of 30 mm and a length of 280 mm in the rolling direction (L-direction) and in a direction perpendicular to the rolling direction (C-direction) as a longitudinal direction, respectively, and the magnetic flux density B₅₀ (T) and iron loss W_{10/400} (W/kg) thereof are measured by a 25 cm Epstein method described in JIS C2550, results of which are also shown in Table1.

**Table 1-1**

| Nº | Chemical composition (mass%) ***** | | | | | | | | | | | | Thickness (mm) | Finish annealing temperature (°C)×10s | Magnetic properties | | Remarks |
|---|---|---|---|---|---|---|---|---|---|---|---|---|---|---|---|---|---|
| | C | Si | Mn | Al | N | P | S | Se | Sn | Sb | Ca | Mg | | | Iron loss W_{10/400} (W/kg) | Magnetic flux density B₅₀(T) | |
| 1 | 0.0019 | 3.01 | 0.15 | 0.0010 | 0.0018 | 0.010 | 0.0005 | 0.0001 | 0.0020 | 0.0001 | 0.0001 | 0.0001 | 0.20 | 980 | 12.00 | 1.65 | Comparative Example |
| 2 | 0.0017 | 3.05 | 0.10 | 0.0010 | 0.0017 | 0.034 | 0.0005 | 0.0001 | 0.0020 | 0.0001 | 0.0001 | 0.0001 | 0.20 | 980 | 12.00 | 1.67 | Comparative Example |
| 3 | 0.0012 | 3.04 | 0.12 | 0.0010 | 0.0012 | 0.051 | 0.0004 | 0.0001 | 0.0020 | 0.0001 | 0.0001 | 0.0001 | 0.20 | 980 | 12.00 | 1.68 | Comparative Example |
| 4 | 0.0013 | 3.04 | 0.12 | 0.0010 | 0.0016 | 0.050 | 0.0015 | 0.0001 | 0.0020 | 0.0001 | 0.0001 | 0.0001 | 0.20 | 980 | 11.90 | 1.68 | Comparative Example |
| 5 | 0.0018 | 3.05 | 0.13 | 0.0020 | 0.0017 | 0.050 | 0.0015 | 0.0001 | 0.0020 | 0.0001 | 0.0001 | 0.0001 | 0.20 | 980 | 11.80 | 1.68 | Comparative Example |
| 6 | 0.0020 | 3.00 | 0.12 | 0.0010 | 0.0019 | 0.100 | 0.0005 | 0.0001 | 0.0020 | 0.0001 | 0.0001 | 0.0001 | 0.20 | 980 | 11.80 | 1.68 | Comparative Example |
| 7 | 0.0017 | 3.01 | 0.15 | 0.0010 | 0.0018 | 0.010 | 0.0005 | 0.0001 | 0.0300 | 0.0001 | 0.0001 | 0.0001 | 0.15 | 980 | 10.00 | 1.65 | Comparative Example |
| 8 | 0.0015 | 3.04 | 0.12 | 0.0010 | 0.0013 | 0.050 | 0.0004 | 0.0001 | 0.0300 | 0.0001 | 0.0001 | 0.0001 | 0.15 | 980 | 9.90 | 1.69 | Comparative Example |
| 9 | 0.0017 | 3.01 | 0.15 | 0.0010 | 0.0018 | 0.010 | 0.0005 | 0.0001 | 0.0300 | 0.0001 | 0.0001 | 0.0001 | 0.10 | 980 | 8.41 | 1.63 | Comparative Example |
| 10 | 0.0021 | 3.04 | 0.12 | 0.0010 | 0.0013 | 0.050 | 0.0004 | 0.0001 | 0.0300 | 0.0001 | 0.0001 | 0.0001 | 0.10 | 980 | 8.35 | 1.68 | Comparative Example |
| 11 | 0.0022 | 3.01 | 0.15 | 0.0010 | 0.0018 | 0.010 | 0.0005 | 0.0001 | 0.0300 | 0.0001 | 0.0001 | 0.0001 | 0.05 | 980 | 7.32 | 1.62 | Comparative Example |
| 12 | 0.0019 | 3.04 | 0.12 | 0.0010 | 0.0013 | 0.050 | 0.0004 | 0.0001 | 0.0300 | 0.0001 | 0.0001 | 0.0001 | 0.05 | 980 | 7.25 | 1.67 | Comparative Example |
| 13 | 0.0020 | 2.81 | 0.16 | 0.0050 | 0.0014 | 0.050 | 0.0005 | 0.0001 | 0.0020 | 0.0001 | 0.0001 | 0.0001 | 0.20 | 980 | 12.90 | 1.65 | Comparative Example |
| 14 | 0.0017 | 2.82 | 0.18 | 0.3000 | 0.0012 | 0.050 | 0.0005 | 0.0001 | 0.0020 | 0.0001 | 0.0001 | 0.0001 | 0.20 | 980 | 12.10 | 1.64 | Comparative Example |
| 15 | 0.0012 | 3.01 | 0.14 | 0.0010 | 0.0018 | 0.050 | 0.0005 | 0.0005 | 0.0020 | 0.0001 | 0.0001 | 0.0001 | 0.20 | 980 | 12.10 | 1.69 | Comparative Example |
| 16 | 0.0013 | 3.00 | 0.21 | 0.0010 | 0.0018 | 0.050 | 0.0005 | 0.0017 | 0.0020 | 0.0001 | 0.0001 | 0.0001 | 0.20 | 980 | 12.20 | 1.68 | Comparative Example |
| 17 | 0.0013 | 3.00 | 0.21 | 0.0010 | 0.0018 | 0.050 | 0.0005 | 0.0025 | 0.0020 | 0.0001 | 0.0001 | 0.0001 | 0.20 | 980 | 12.40 | 1.66 | Comparative Example |
| 18 | 0.0018 | 3.00 | 0.21 | 0.0010 | 0.0020 | 0.050 | 0.0005 | 0.0043 | 0.0020 | 0.0001 | 0.0001 | 0.0001 | 0.20 | 980 | 12.50 | 1.66 | Comparative Example |
| 19 | 0.0022 | 2.80 | 0.21 | 0.3000 | 0.0023 | 0.050 | 0.0005 | 0.0001 | 0.0020 | 0.0001 | 0.0001 | 0.0001 | 0.20 | 980 | 12.10 | 1.64 | Comparative Example |
| 20 | 0.0012 | 3.04 | 0.21 | 0.0010 | 0.0012 | 0.050 | 0.0005 | 0.0001 | 0.0020 | 0.0020 | 0.0001 | 0.0001 | 0.20 | 980 | 11.80 | 1.68 | Comparative Example |

**Table 1-2**

| Nº | Chemical composition (mass%) * | | | | | | | | | | | | Thickness (mm) | Finish Annealing temperature (°C)×10s | Magnetic properties | | Remarks |
|---|---|---|---|---|---|---|---|---|---|---|---|---|---|---|---|---|---|
| | C | Si | Mn | Al | N | P | S | Se | Sn | Sb | Ca | Mg | | | Iron loss W_{10/400} (W/kg) | Magnetic flux density B₅₀(T) | |
| 21 | 0.0015 | 3.10 | 0.20 | 0.0010 | 0.0025 | 0.050 | 0.0005 | 0.0001 | 0.0020 | 0.0300 | 0.0001 | 0.0001 | 0.20 | 980 | 11.60 | 1.69 | Comparative Example |
| 22 | 0.0016 | 3.00 | 0.18 | 0.0010 | 0.0012 | 0.050 | 0.0005 | 0.0001 | 0.0025 | 0.0001 | 0.0001 | 0.0001 | 0.20 | 980 | 11.80 | 1.68 | Comparative Example |
| 23 | 0.0014 | 3.05 | 0.17 | 0.0010 | 0.0019 | 0.050 | 0.0005 | 0.0001 | 0.0100 | 0.0001 | 0.0001 | 0.0001 | 0.20 | 980 | 11.70 | 1.69 | Comparative Example |
| 24 | 0.0013 | 3.09 | 0.21 | 0.0010 | 0.0011 | 0.050 | 0.0005 | 0.0001 | 0.0500 | 0.0001 | 0.0001 | 0.0001 | 0.20 | 980 | 11.50 | 1.69 | Comparative Example |
| 25 | 0.0019 | 2.99 | 0.21 | 0.0010 | 0.0019 | 0.050 | 0.0025 | 0.0001 | 0.0001 | 0.0001 | 0.0001 | 0.0001 | 0.20 | 980 | 12.00 | 1.67 | Comparative Example |
| 26 | 0.0019 | 3.00 | 0.20 | 0.0010 | 0.0018 | 0.050 | 0.0025 | 0.0001 | 0.0001 | 0.0001 | 0.0020 | 0.0001 | 0.20 | 980 | 11.90 | 1.68 | Comparative Example |
| 27 | 0.0020 | 3.00 | 0.21 | 0.0010 | 0.0022 | 0.050 | 0.0025 | 0.0001 | 0.0001 | 0.0001 | 0.0001 | 0.0020 | 0.20 | 980 | 11.90 | 1.68 | Invention Example |
| 28 | 0.0125 | 3.01 | 0.23 | 0.0010 | 0.0013 | 0.050 | 0.0005 | 0.0001 | 0.0020 | 0.0001 | 0.0001 | 0.0001 | 0.20 | 980 | 12.60 | 1.66 | Comparative Example |
| 29 | 0.0021 | 0.70 | 0.19 | 0.0010 | 0.0018 | 0.050 | 0.0005 | 0.0001 | 0.0020 | 0.0001 | 0.0001 | 0.0001 | 0.20 | 980 | 14.90 | 1.74 | Comparative Example |
| 30 | 0.0020 | 1.20 | 0.21 | 0.0010 | 0.0020 | 0.050 | 0.0005 | 0.0001 | 0.0020 | 0.0001 | 0.0001 | 0.0001 | 0.20 | 980 | 13.80 | 1.73 | Comparative Example |
| 31 | 0.0016 | 2.00 | 0.21 | 0.0010 | 0.0023 | 0.050 | 0.0005 | 0.0001 | 0.0020 | 0.0001 | 0.0001 | 0.0001 | 0.20 | 980 | 12.70 | 1.72 | Comparative Example |
| 32 | 0.0012 | 4.51 | 0.21 | 0.0010 | 0.0012 | 0.050 | 0.0005 | 0.0001 | 0.0020 | 0.0001 | 0.0001 | 0.0001 | 0.20 | 980 | 10.80 | 1.65 | Comparative Example |
| 33 | 0.0013 | 3.00 | 1.20 | 0.0010 | 0.0016 | 0.050 | 0.0005 | 0.0001 | 0.0020 | 0.0001 | 0.0001 | 0.0001 | 0.20 | 980 | 11.40 | 1.68 | Comparative Example |
| 34 | 0.0013 | 3.00 | 1.60 | 0.0010 | 0.0016 | 0.050 | 0.0005 | 0.0001 | 0.0020 | 0.0001 | 0.0001 | 0.0001 | 0.20 | 980 | 10.90 | 1.67 | Comparative Example |
| 35 | 0.0019 | 3.01 | 3.50 | 0.0010 | 0.0012 | 0.050 | 0.0005 | 0.0001 | 0.0020 | 0.0001 | 0.0001 | 0.0001 | 0.20 | 980 | 11.50 | 1.65 | Comparative Example |
| 36 | 0.0022 | 3.00 | 0.21 | 0.0010 | 0.0062 | 0.050 | 0.0020 | 0.0001 | 0.0020 | 0.0001 | 0.0001 | 0.0001 | 0.20 | 980 | 12.90 | 1.65 | Comparative Example |
| 37 | 0.0021 | 3.00 | 0.21 | 0.0010 | 0.0020 | 0.050 | 0.0150 | 0.0001 | 0.0020 | 0.0001 | 0.0001 | 0.0001 | 0.20 | 980 | 13.10 | 1.64 | Comparative Example |

As seen from Table 1, the non-oriented electrical steel sheets according to the invention having ingredients of Al, P and Se adjusted to acceptable ranges are high in the magnetic flux density and excellent in the iron loss property as compared to steel sheets of the comparative examples having the ingredients outside the ranges.

### INDUSTRIAL APPLICABILITY

The non-oriented electrical steel sheets according to the invention are applicable to an electric power steering motor, a hard disk motor for an information device and so on.

## Claims

1. A non-oriented electrical steel sheet having a chemical composition consisting of C: not more than 0.010 mass%, Si: 1-4 mass%, Mn: 0.05-3 mass%, Al: not more than 0.004 mass%, N: not more than 0.005 mass%, P: 0.03-0.20 mass%, S: not more than 0.01 mass%, Se: not more than 0.002 mass%, Mg: 0.001-0.005 mass%, optionally Ca: 0.001-0.005 mass%, and the remainder being Fe and inevitable impurities.

2. A non-oriented electrical steel sheet having a chemical composition consisting of C: not more than 0.010 mass%, Si: 1-4 mass%, Mn: 0.05-3 mass%, Al: not more than 0.004 mass%, N: not more than 0.005 mass%, P: 0.03-0.20 mass%, S: not more than 0.01 mass%, Se: not more than 0.003 mass%, one or two of Sn: 0.001-0.1 mass% and Sb: 0.001-0.1 mass%, Mg: 0.001-0.005 mass%, optionally Ca: 0.001-0.005 mass%, and the remainder being Fe and inevitable impurities.

3. The non-oriented electrical steel sheet according to claims 1 or 2, wherein a thickness is 0.05-0.30 mm.

## Patentansprüche

1. Ungerichtetes Elektrostahlblech mit einer chemischen Zusammensetzung bestehend aus C: nicht mehr als 0,010 Masse%, Si: 1-4 Masse%, Mn: 0,05-3 Masse%, Al: nicht mehr als 0,004 Masse%, N: nicht mehr als 0,005 Masse%, P: 0,03-0,20 Masse%, S: nicht mehr als 0,01 Masse%, Se: nicht mehr als 0,002 Masse%, Mg: 0,001-0,005 Masse%, optional Ca: 0,001-0,005 Masse%, wobei es sich bei dem Rest um Fe und unvermeidbare Verunreinigungen handelt.

2. Ungerichtetes Elektrostahlblech mit einer chemischen Zusammensetzung bestehend aus C: nicht mehr als 0,010 Masse%, Si: 1-4 Masse%, Mn: 0,05-3 Masse%, Al: nicht mehr als 0,004 Masse%, N: nicht mehr als 0,005 Masse%, P: 0,03-0,20 Masse%, S: nicht mehr als 0,01 Masse%, Se: nicht mehr als 0,003 Masse%, einem oder zwei von Sn: 0,001-0,1 Masse% und Sb: 0,001-0,1 Masse%, Mg: 0,001-0,005 Masse%, optional Ca: 0,001-0,005 Masse%, wobei es sich bei dem Rest um Fe und unvermeidbare Verunreinigungen handelt.

3. Ungerichtetes Elektrostahlblech nach den Ansprüchen 1 oder 2, wobei eine Dicke 0,05-0,30 mm beträgt.

## Revendications

1. Une tôle d'acier électrique non orientée présentant une composition chimique composée de C : pas plus de 0,010 % en masse, Si : 1 à 4 % en masse, Mn : 0,05 à 3 % en masse, Al : pas plus de 0,004 % en masse, N : pas plus de 0,005 % en masse, P : 0,03 à 0,20 % en masse, S : pas plus de 0,01 % en masse, Se: pas plus de 0,002 % en masse, Mg : 0,001 à 0,005 % en masse, éventuellement Ca : 0,001 à 0,005 % en masse et le reste étant le Fe et des impuretés inévitables.

2. Une tôle d'acier électrique non orientée présentant une composition chimique composée de C : pas plus de 0,010 % en masse, Si : 1 à 4 % en masse, Mn : 0,05 à 3 % en masse, Al : pas plus de 0,004 % en masse, N : pas plus de 0,005 % en masse, P : 0,03 à 0,20 % en masse, S : pas plus de 0,01 % en masse, Se: pas plus de 0,003 % en masse, un ou deux parmi Sn : 0,001 à 0.1 % en masse et Sb : 0,001 à 0,1 % en masse, Mg: 0,001 à 0,005 % en masse, éventuellement Ca: 0,001 à 0,005 % en masse et le reste étant le Fe et des impuretés inévitables.

3. La tôle d'acier électrique non orientée selon les revendications 1 ou 2, dans laquelle une épaisseur est de 0,05 à 0,30 mm.
